

1,155,861.

L. A. WOOD.  
ORE CONCENTRATION.  
APPLICATION FILED JUNE 2, 1914.

Patented Oct. 5, 1915.



*Witnesses*

Mr. Ashley Kelley  
Kenneth D.D. Adams

Inventor  
Louis Albert Wood

By Henry D. Williams  
Attorney.

# UNITED STATES PATENT OFFICE.

LOUIS ALBERT WOOD, OF LONDON, ENGLAND, ASSIGNOR TO MINERALS SEPARATION  
AMERICAN SYNDICATE (1913) LIMITED, OF LONDON, ENGLAND.

## ORE CONCENTRATION.

1,155,861.

Specification of Letters Patent.

Patented Oct. 5, 1915.

Application filed June 2, 1914. Serial No. 842,449.

To all whom it may concern:

Be it known that I, LOUIS ALBERT WOOD, a subject of the King of England, residing at London, in England, have invented certain 5 new and useful Improvements in Ore Concentration, of which the following is a specification.

This invention is for improvements in or relating to ore concentration the object being 10 to simplify both the process and the apparatus for concentrating ores by gaseous selection.

In the agitation froth process as commonly worked and as described for example 15 in the United States Patent No. 835120 granted November 6th, 1906, the finely powdered ore is suspended in acidified water containing a small proportion of an oily 20 substance and the pulp is agitated so as to beat into it the supernatant air whereby a froth is formed containing the metalliferous matter. There have been many modifications 25 of the agitation froth process such as the replacement of the oil by other frothing agents, in some cases soluble in water. It has also been proposed to dispense with the use of acid in certain cases or to employ other chemical agents.

Again, in processes of the Potter type as 30 described for example in United States Patent No. 776145, granted November 29th, 1904, the finely powdered ore is mixed with water containing sulfuric acid and heat is applied in such a way as to bring about the 35 chemical evolution of gaseous bubbles in the pulp, the evolved bubbles attaching themselves preferentially to certain metalliferous particles and rising and floating on the surface.

40 Various types of apparatus have been devised for carrying these processes into effect, for example United States Patent No. 763749 granted June 28th, 1904, describes a method and apparatus for carrying out the 45 Potter process in which the minerals in the finely divided condition are subjected to the action of an acidulated solution which results in the formation of gas bubbles to which certain particles of the minerals adhere, the said mineral loaded bubbles being directed upwardly to the surface of the solution where they burst and release said particles which are thereupon precipitated and 50 collected in suitable troughs.

55 In United States Patent No. 1093463

granted April 14th, 1914, are described a method and apparatus for concentrating ores by gaseous flotation of certain mineral particles in liquid in which the agitation froth as it is formed is caused to fall over a trap 60 or wall below the level of the free air surface whereby the froth is collected and removed from the pulp before the bubbles can burst.

Hitherto it has been known that without 65 the use of any oil or other frothing agent, and without necessarily using acid or heat, sulfid particles in an aqueous pulp would preferentially attach to themselves bubbles or films of air which have been suitably introduced into the pulp and that such sulfid particles could be raised to the surface by bubbles or films or air. Such bubbles with the associated mineral do not readily form 70 a persistent and coherent froth and the 75 phenomenon has not therefore received any practical embodiment.

According to this invention a pulp consisting of powdered ore freely suspended in water is subjected to the admission of gas 80 or a mixture of gases such as air which is disseminated in such a way that the gaseous 85 films or bubbles preferentially attach themselves to the metalliferous particles such as sulfids and rise toward the surface of the liquid. The ore pulp to which the air is admitted may according to this invention 90 be subjected to agitation. When the bubbles at or near the surface of the liquid discharge the mineral the latter is caught in a trough 95 below the level of the liquid.

The accompanying drawings illustrate 100 diagrammatically a suitable apparatus for carrying this invention into effect, which consists of an upright vessel A preferably 105 rectangular having an inlet for air B at the bottom, with a valve B<sup>1</sup> in the inlet conduit. The vessel A is provided at the bottom with an agitating device such as a propeller C. Above the propeller, baffles D may be provided to bring the pulp to a state of comparative rest. Above these baffles, but below the surface of the pulp, is placed an inclined plate or deflector E extending across the vessel and horizontal liquid surface F, the arrangement being such that air is introduced under pressure or otherwise into the pulp which is then agitated so as to bring 110 the finely divided air into contact with the suspended ore particles whereupon the gase-

- ous bubbles with the associated particles rise toward or to the surface of the liquid, depositing the mineral into the trough or receiver formed by the plate or deflector E under the surface of the liquid. Suitable means may be provided for removing the selected particles intermittently or continuously, for example the vessel may be provided at the bottom of the trough with an outlet G leading to a concentrate launder G<sup>1</sup>. The ore pulp may be fed to the vessel through the inlet H and the tailing ore pulp which has been depleted of certain mineral contents may be removed through the outlet J.
15. In the example of apparatus illustrated there is one plate E forming a trough to receive the concentrates, but two or more such plates may be used or the apparatus may be otherwise arranged in such a way that when the 20 gaseous bubbles at or near the surface of the liquid discharge the associated mineral, the latter is caught in a trough or receiver below the level of the liquid.

The following are examples of the practical application of this invention.

25 A powdered ore containing copper sulfid was mixed with water at ordinary temperature and without any addition of frothing agent or chemical agent. The pulp was subjected to agitation and aeration in an apparatus of the type described and it was found that the bubbles of air selected the particles of copper sulfid and raised them toward or to the surface of the liquid where the bubbles discharged the associated mineral into the receiving trough from which they were removed, an efficient separation of the values from the gangue being thus obtained. Again, Broken Hill tailings crushed to 60 mesh 30 were mixed with four times their weight of water at atmospheric temperature containing about 1% of sulfuric acid on the weight of ore. This pulp was subjected to agitation and aeration as above described and a good 35 recovery of zinc and lead sulfids of a high grade was obtained. In some cases it was found advantageous to heat the pulp to a temperature of 50° to 60° C. The use of oil or any other frothing agent is avoided as 40 such use under the conditions specified tends to result in the formation of a more or less persistent and coherent froth, whereas according to this invention the formation of such a froth is avoided. Examples have been 45 given for the separation of sulfids from gangue but the method and apparatus are applicable also to the separation of different sulfids from one another as well as from gangue. The conditions such as the amount 50 of aeration have to be varied according to the nature of the ore and the degree of crushing and a simple preliminary test is necessary to determine the best conditions for the treatment of any particular ore.

What I claim as my invention and desire 65 to secure by Letters Patent is:—

1. A process of concentrating ores which consists in subjecting the powdered ore suspended in water free from frothing agents to the admission of gas, forcefully disseminating the gas through the pulp in such a way that the gaseous bubbles preferentially attach themselves to certain mineral particles and rise toward the surface and discharge their mineral load within the pulp, 75 and catching and removing such discharged mineral below the surface of the liquid.

2. A process of concentrating ores, which consists in introducing gas to the lower zone of an ore pulp free from frothing agents, 80 subjecting such ore pulp in its lower zone to agitation whereby the gas will be forcefully disseminated through the pulp, maintaining the upper zone of the pulp in a state of comparative quiescence, whereby gas bubbles attach themselves selectively to certain mineral particles and rise toward the surface and discharge their mineral load within the pulp, 85 and catching and removing such discharged mineral below the surface of the 90 liquid.

3. A process of concentrating ores which consists in subjecting a liquid mass of ore pulp free from frothing agents to continuous agitation in its lower zone, introducing 95 fresh ore pulp continuously to said liquid mass, removing depleted ore pulp continuously from said liquid mass, introducing gas continuously to the lower zone of the pulp so that it will be forcefully disseminated 100 through the pulp by the agitation of the pulp in the lower zone thereof, maintaining the upper zone of the pulp in a state of comparative quiescence, whereby gaseous bubbles attach themselves selectively to certain mineral particles and rise toward the surface and discharge their mineral load within the pulp, 105 and catching and removing such discharged mineral below the surface of the liquid.

4. A process of concentrating sulfid ores which consists in subjecting the powdered ore suspended in water free from frothing agents to the admission of air, forcefully disseminating the air through the pulp in 115 such a way that the air bubbles preferentially attach themselves to certain sulfid particles and rise toward the surface and discharge their mineral load in the pulp, and catching and removing such discharged mineral below the surface of the liquid.

5. A process of concentrating sulfid ores which consists in subjecting the liquid mass of ore pulp free from frothing agents to agitation in its lower zone, introducing air to 125 the lower zone of the pulp so that it will be forcefully disseminated through the pulp by the agitation of the lower zone thereof, ob-

structing the turbulence of the pulp in its upper zone, whereby air bubbles attach themselves selectively to certain sulfid particles and rise toward the surface and discharge their load of sulfid particles within the pulp, and catching and removing said discharged sulfid particles below the surface of the liquid.

6. A process of concentrating sulfid ores which consists in subjecting a liquid mass of ore pulp free from frothing agents to continuous agitation in its lower zone, introducing fresh ore pulp continuously to said liquid mass, and removing depleted ore pulp continuously from said liquid mass, introducing air continuously to the lower zone of the pulp so that it will be forcefully dis-

seminated through the pulp by the agitation of the lower zone thereof, obstructing the turbulence of the pulp in its upper zone, 20 whereby air bubbles attach themselves selectively to certain sulfid particles and rise toward the surface and discharge their load of sulfid particles within the pulp, and catching and removing such discharged sulfid particles below the surface of the liquid. 25

In testimony whereof I have signed my name to this specification in the presence of two subscribing witnesses.

LOUIS ALBERT WOOD.

Witnesses:

WILLIAM H. BALLANTYNE,  
HARRY B. BLIDGE.